

Feb. 2, 1943.

R. F. RUTHRUFF

2,309,987

MOTOR FUEL AND PREPARATION THEREOF

Filed Nov. 15, 1939



## UNITED STATES PATENT OFFICE

2,309,987

## MOTOR FUEL AND PREPARATION THEREOF

Robert F. Ruthruff, Chicago, Ill.

Application November 15, 1939, Serial No. 304,602

4 Claims. (Cl. 196—10)

This invention relates to motor fuel and the preparation thereof. More particularly, this invention relates to motor fuel of high octane number and controllable volatility and the preparation thereof.

During the last few years the steady improvement in motor fuel quality as regards octane number, volatility and other characteristics is too well known to those skilled in the art to merit further discussion. While the possible limits to such improvements have not as yet been approached in all probability, nevertheless, in certain directions, additional improvements are becoming increasingly difficult to achieve and all the resources of petroleum technology must be applied to the problem. This is particularly true in the case of high octane motor fuels for aviation use.

In the past, high octane number motor fuels for aviation use have been prepared by the catalytic polymerization of olefines containing four carbon atoms to the molecules followed by hydrogenation of the polymer formed. Such olefines may be obtained, in admixture with the analogous paraffins, from the gases produced during the cracking of various petroleum fractions or by the catalytic dehydrogenation or the thermal pyrolysis of the butane cut from natural gas. These olefines consist of isobutene and the normal butenes. When such a mixture is passed over a suitable catalyst under suitable conditions as regards to temperature, pressure and time of contact, polymerization occurs. In this reaction the isobutene reacts very rapidly while the normal butenes react at a much slower rate. By the proper selection of operating conditions it is possible to attain almost quantitative conversions of isobutene to polymer with conversions of normal butenes varying from practically zero to practically 100%. The polymer produced consists largely of isomeric octenes and has an octane number of 80 to 82. While an excellent motor fuel for automobile engines, this material is totally unsuited for aviation uses because of its high unsaturate content, low octane number and low lead response. By catalytic hydrogenation the polymer may be converted to iso-octanes having an octane number of 90 to 98. The hydrogenated material is completely saturated and exhibits an excellent lead response. The octane number of the hydrogenated polymer is largely a function of the amount of normal butenes reacting. When the ratio of reacting isobutene to reacting normal butenes is high the

octane number of the resulting hydrogenated polymer is high and vice versa.

While the hydrogenated catalytic polymer shows considerable promise as a high octane number aviation fuel and has been much used for the purpose, yet the material and the process for preparing the same exhibits numerous disadvantages. For example, the hydrogenated catalytic polymer is not sufficiently volatile for aviation requirements, the unhydrogenated polymer obviously suffering from the same disadvantage. If an attempt is made to increase volatility by the addition of light naphthas the octane number of the blend is considerable lower than that shown by the straight hydrogenated polymer. Furthermore, the possible yield of hydrogenated polymer is quite low. It is obvious that the yield can be no higher than the olefines present in the charge and actually, if a high octane product is desired, is usually much less. If a high octane hydrogenated catalytic polymer is to be made it is well to react not more than one mole of normal butenes per mole of isobutene present. However, as is well known to those skilled in the art, the isobutane-normal butane ratio in natural gas and the isobutene-normal butenes ratio in cracked gas is much less than unity so if it is desired to make a hydrogenated catalytic polymer of the highest octane number considerable normal butenes must be discarded.

In order to eliminate or reduce normal butenes discard during catalytic polymerization and at the same time produce a polymer exhibiting a high octane number after hydrogenation it is obvious that additional isobutene must be added to the charge to the polymerizer. It has been suggested that this additional isobutene be obtained by isomerizing normal butane to isobutane followed by catalytic dehydrogenation or thermal pyrolysis of the isobutane to produce isobutene. While this procedure solves the particular problems mentioned, it is obvious that the volatility deficiency of the hydrogenated polymer still remains.

Many attempts have been made to increase the volatility of iso-octanes formed by the catalytic hydrogenation of catalytic polymer. Since isopentane is the only low boiling liquid isoparaffin readily available, isopentane-iso-octane blends have been proposed as aviation fuels. As those skilled in the art are aware, aviation fuels meeting current specifications cannot be prepared in this way. If the blend meets the 10% off specification, the 50% off specification is not satisfied. Likewise, if the blend has the proper

amount of isopentane to satisfy the 50% off specification, the minimum permissible temperature for 10% off is far exceeded. To correct for these deficiencies, light naphtha has been added to the isopentane-isoctane blend. When this is done the octane number is very much below that shown by the straight isoctane. Very recently, dimethyl butane (2,2) has been suggested as a blending agent for isoctane, with or without isopentane. While the use of this compound as a blending agent results in considerable improvement the fact remains that this hexane is very difficult to obtain. At present this material is made by the thermal alkylation of isobutane with ethene at extremely high pressures. To reduce ethene polymerization, the concentration of this olefine must be kept at an extremely low level. This means that the yield per pass of the desired compound is very low, which in turn necessitates an extremely high recycle ratio and the separation of the small amount of the isomeric hexane from a large amount of unreacted material.

One object of this invention is to provide an improved motor fuel and a process for producing the same. A further object of this invention is to provide an improved motor fuel of high octane number and a process for producing the same. An additional object of this invention is to provide an improved motor fuel of controlled volatility and a process for producing the same. Another object of this invention is to provide an improved motor fuel of high octane number and controlled volatility and a process for producing the same. Further objects of this invention will become evident from the following description.

Briefly, the improved motor fuel of the instant invention comprises hydrogenated catalytic polymer blended with a light naphtha of high isoparaffin content obtained by the destructive isomerization of a hydrocarbon fraction. (Destructive isomerization is defined immediately hereinafter.) The hydrogenated catalytic polymer is prepared by catalytically polymerizing a mixture containing isobutene, at least part of said isobutene being derived from the catalytic dehydrogenation or thermal pyrolysis of isobutane obtained by the destructive isomerization of a hydrocarbon fraction, followed by the catalytic hydrogenation of the polymer produced. The resulting hydrogenated catalytic polymer is blended with a light naphtha of high volatility and high isoparaffin content, and hence of high octane number, at least part of which was also obtained by the destructive isomerization of a hydrocarbon fraction. The blend comprises a motor fuel of very low unsaturate content, high octane number, high lead response and high and controllable volatility. In the production of this material the processes of destructive isomerization, catalytic polymerization, catalytic hydrogenation and catalytic dehydrogenation (or thermal pyrolysis) co-operate to produce a new and unexpected result as will become manifest from the following description.

For a description of the process of destructive isomerization reference may be made to my United States application, Serial Number 2,379, filed July 20, 1935, and which has since matured into United States Patent 2,172,146, issued September 5, 1939. In this it is shown that when a hydrocarbon fraction, for example a straight run heavy naphtha, is treated at low temperatures, for example, 205-210° F., with a suitable catalyst, for example aluminum chloride promoted with water, hydrogen chloride, carbon

tetrachloride or the like, a large part of the hydrocarbon fraction charged is converted into gaseous products and these consist almost exclusively of isobutane.

To this process the term destructive isomerization is applied. Isomerization is used to designate reactions wherein a compound is converted into a second compound having the same chemical composition and molecular weight but different structure than that of the first. The classical synthesis of urea from ammonium cyanate and the conversion of normal butane to isobutane are examples of isomerization. In the present instance however, in addition to forming a compound of different structure than that of the charge, the new compound also has a different molecular weight. In the example cited, a considerable amount of heavy naphtha charge, having an average molecular weight of say 142, is converted into isobutane having a molecular weight of 58. In other words, in this reaction, the charge was first decomposed and the resulting fragments were then isomerized—hence the term destructive isomerization.

It might be argued that the above reaction was entirely one of destruction without any isomerization. For example, it might be argued with no little merit that the isobutane resulted from the preferential decomposition of 2-methyl paraffins between carbon atoms 3 and 4. In this way isobutane could be formed without any isomerization. A mass of experimental data shows that this stand is not tenable. For example, in the example cited, Mt. Pleasant heavy naphtha was used as charge. As is well known to those skilled in the art, this material consists largely of straight chain paraffins. In addition, this stock was heavily acid treated before use so as to remove aromatics and similar compounds, so as charged it consisted essentially of a mixture of straight chain paraffins.

Supplementary experiments have also confirmed the fact that straight chain paraffins are destructively isomerized with the production of isobutane. For example, a heavily acid treated Mt. Pleasant heavy naphtha was exhaustively treated with chlorosulfonic acid. This last named reagent removes hydrocarbons having tertiary carbon atoms. Upon subjecting the thus treated material to destructive isomerization as before, large amounts of isobutane formed. Furthermore, synthetic normal heptane and synthetic normal heptane after exhaustive treatment with chlorosulfonic acid as previously described, when subjected to destructive isomerization gave isobutane in greater yields and with greater ease than Mt. Pleasant heavy naphtha.

A further study of the products of destructive isomerization has revealed a most important but hitherto unnoticed fact. On fractionating the products obtained by the destructive isomerization of a heavy naphtha for example, one cut may be obtained representing the isobutane produced and a second containing a material boiling from above isobutane up to the endpoint of the heavy naphtha charge. The octane number of this second cut has been found to be materially higher than that of the heavy naphtha charge. As is well known to those skilled in the art, octane number increases as volatility increases. To evaluate the effect of volatility on octane number increase observed, this second cut was again distilled, taking overhead a fraction boiling from above isobutane up to the initial of the naphtha charge and leaving as bottoms

a material having approximately the same boiling range as the heavy naphtha charge. On determining the octane numbers of the two fractions thus made it was found that the bottoms had an octane number not greatly different than that of the original heavy naphtha charge, while the light naphtha overhead had an extremely high octane number. It is apparent that the reaction is predominantly one of destructive isomerization only, any parts of the original charge escaping destructive isomerization are not affected to any great extent. In a large number of experiments the light naphtha overhead had octane numbers averaging 80 motor, some 15 to 20 units higher than that of an East Texas light naphtha of the same boiling range. Investigation showed that the light naphtha formed during destructive isomerization of the hydrocarbon fractions consisted largely of isoparaffins, these accounting for the unusually high octane numbers observed.

To summarize, in the destructive isomerization of heavy naphtha the following major products are obtained:

- A. Isobutane.
- B. Light naphtha of very high octane number and consisting largely of isoparaffins.
- C. Heavy naphtha of the same boiling range and approximately the same octane number as the charge.
- D. Material having a higher boiling point than that of the charge.

It will be evident to those skilled in the art that the process of destructive isomerization differs materially from both thermal reforming and catalytic reforming. In thermal reforming, the gas formed contains all gaseous paraffins and olefines together with hydrogen. In destructive isomerization the gas consists essentially of isobutane. In thermal reforming, the light naphtha produced is highly unsaturated. The light naphtha obtained in destructive isomerization operations is completely saturated or nearly so. The product from thermal reforming having the same boiling range as that of the charge is highly olefinic and has a much higher octane number than that of the charge. The same fraction from destructive isomerization contains no olefines or practically none and has an octane number differing little from that of the original charge. In catalytic reforming, the gas produced consists largely of hydrogen, very little light naphtha is produced and the material having the same boiling range as that of the charge consists largely of aromatic hydrocarbons.

The catalytic polymerization-hydrogenation process for the production of higher isoparaffins is so well known to those skilled in the art that only the briefest mention is necessary. In the catalytic polymerization step a mixture containing olefines is contacted with a suitable catalyst, such as phosphoric acid on carbon, usually at elevated to high superatmospheric pressures and moderate temperatures. Usually gas mixtures comprising hydrocarbons containing four carbon atoms to the molecule are employed, the isobutene and normal butenes present polymerizing to form isoctenes. The resulting polymer is then catalytically hydrogenated, usually at moderate temperatures and pressures in the presence of a highly active hydrogenation catalyst, for example, nickel, to form isoctanes, the resulting product having a very low unsaturated content, high octane number and a high lead response, all these properties being much desired

in aviation fuels. However, as has been mentioned previously, the hydrogenated polymer is not sufficiently volatile for use as an aviation fuel and when blended with the light naphthas ordinarily available the octane number of the blend is appreciably lower than that of the straight hydrogenated polymer. Also, the manufacture of hydrogenated polymer is not efficient because of the dearth of isobutene. In the ordinary refinery the yield of high octane number hydrogenated polymer could be increased two or more fold were sufficient isobutene available to give, for example, an amount equal in volume to the normal butenes at hand.

The excellent cooperation between destructive isomerization and catalytic polymerization-hydrogenation for the manufacture of high octane motor fuels for aviation use, should now be evident. For maximum production of high octane number hydrogenated polymer, additional isobutene over that found in the usual refinery is required. Destructive isomerization supplies isobutane which is easily converted to isobutene by catalytic dehydrogenation or thermal pyrolysis. To confer proper volatility on the hydrogenated polymer without at the same time greatly lowering the octane number shown by the straight hydrogenated polymer, a light naphtha of high octane number is required. Destructive isomerization furnishes such a light naphtha. Also in the conversion of isobutane required in the catalytic polymerization reaction, hydrogen is produced as a by-product while in the conversion of catalytic polymer into iso-octane hydrogen is required.

While the specific details of the destructive isomerization process and of the catalytic polymerization-hydrogenation process, such as temperature, pressures, contact times and catalysts, form no part of the instant invention, some discussion of these details will be included to aid those skilled in the art to select processes best suited to any particular set of conditions.

With respect to destructive isomerization, a wide variety of hydrocarbon fractions may be used as charging stocks. A particularly suitable charging stock for the purpose comprises a virgin heavy naphtha having a boiling range from about 250° F. to 400° F., more or less. Such naphthas as those from East Texas crudes, Mid-Continent crudes and similar average crudes are well suited to the process as are naphthas having an abnormally high amount of normal paraffins such as Michigan naphthas, Pennsylvania naphthas, liquid hydrocarbons produced by the interaction of carbon monoxide and hydrogen (kogasin), raffinates from the solvent extraction of kerosenes and the like. Preferably a light naphtha or a straight run gasoline of normal boiling range is not used as charge for in such cases the high octane number light naphthas formed by destructive isomerization would be diluted with unconverted virgin light naphtha, thus defeating the objects of this invention to a greater or less degree. Also, when aluminum halide type catalysts are employed it is preferable to use an olefine free charge in order to reduce polymer formation to a minimum.

A number of catalysts may be employed to promote the destructive isomerization reaction. Among these may be mentioned aluminum halides, alumina and clays, both natural clays, treated natural clays and synthetic clays. The operating conditions to be employed when oper-

ating at atmospheric pressure and when using aluminum chloride as a catalyst have already been outlined and further details may be obtained by consulting the previously mentioned United States Patent 2,172,146. It has been found that aluminum bromide is much more effective in this reaction than aluminum chloride due to the greater solubility of the former in hydrocarbons.

In place of straight aluminum chloride or bromide, aluminum halides containing various amounts of finely divided metals such as aluminum, magnesium and zinc may be employed. By varying the aluminum halide to metal ratio in the catalyst, the isobutane to light naphtha ratio of the destructively isomerized product may be changed. When large amounts of one of the finely divided metals are incorporated into the halide, isobutane production is largely repressed while light naphtha production is but slightly repressed. On the other hand, with straight aluminum halides the isobutane to light naphtha ratio is maximum. By varying the composition of the catalyst in this manner, isobutane and light naphtha may be produced in any proportions desired. It should be obvious that in any case, the light naphtha formed may be fractionated to give a material of the proper boiling range and volatility for use in the final motor fuel blend and that any excess isobutane over requirements may be discarded.

Destructive isomerization may be conducted batchwise or preferably in a continuous system wherein the charge is passed over any of the various catalysts mentioned or other suitable contacts which may be mounted on supports if desired. Temperature of operation is usually rather low, varying from say 100° F. to 800° F., usually from 200° F. to 700° F. The exact temperature to be employed depends largely upon the catalyst selected. When aluminum halides and similar contacts are used temperatures of from 200° F. to 400° F. may be employed while less active catalysts require higher temperatures, for example in the range 400° F. to 700° F. If desired, the reaction may be conducted under superatmospheric pressure. Actually, because of the rather low velocity of this destructive isomerization reaction, for economy in reactor size and the like it may be desirable to run under high superatmospheric pressure, especially in event that the less active catalysts are employed.

The destructively isomerized product is separated by fractionation or other suitable means into a low boiling isoparaffin cut, usually comprising isobutane, or isobutane and isopentane, a higher boiling isoparaffin cut which may boil from the endpoint of the lower boiling isoparaffinic cut up to the initial boiling point of the hydrocarbon charge, a cut having the same boiling range as the hydrocarbon charge and bottoms having a higher boiling range than the hydrocarbon charge. The cut having the same boiling range as the hydrocarbon charge may be recycled if desired. Or, if desired, the hydrocarbon charge may be added continuously to the reaction vessel for destructive isomerization, product boiling lower than the initial boiling point of the hydrocarbon charge may be taken overhead continuously and separated into a low boiling isoparaffinic cut and a higher boiling isoparaffinic cut. From time to time, or continuously, liquid may be withdrawn from the reactor to prevent accumulation of material boiling higher than the hydrocarbon charge, sludge,

et cetera. If desired, fresh catalyst may be added with the charge to the reactor.

Before turning to a consideration of the catalytic polymerization - hydrogenation reaction proper it will be well to devote a few words to the charging stock employed in the catalytic polymerization step. As has been mentioned previously, at least part of this stock comprises isobutene formed by the catalytic dehydrogenation or thermal pyrolysis of the isobutane produced during destructive isomerization. As the conversion of isobutane to isobutene by catalytic dehydrogenation is preferably employed, the process whereby this change is accomplished by thermal pyrolysis will not be considered. In catalytic dehydrogenation, the isobutane is charged to a reactor containing a highly active dehydrogenating catalyst, for example, chromium oxide on alumina. An operating temperature of from 1000° F. to 1100° F., more or less, may be employed and while theoretically low pressures are preferable, actually moderate superatmospheric pressure, for example, 30 pounds per square inch, may be used without appreciable harm and with considerable savings in reactor cost and the like. Depending upon the space velocity of the charge and the operating temperature, up to 40% or more of the entering isobutane is converted to olefines, about 90% of the olefines produced being isobutene. The resulting product is preferably subjected to a suitable separation process, for example, the well known absorption-fractionation process to remove hydrogen and produce a cut consisting largely of isobutane and isobutene, suitable for charging to the catalytic polymerization unit. If a refinery butane cut is available containing appreciable isobutene and normal butenes, this may be added to the isobutene-isobutane fraction obtained as described heretofore. On the other hand, if a natural gas butane cut is available, mixing this with the isobutane produced by destructive isomerization prior to charging to the catalytic dehydrogenation zone is the obvious and proper procedure. Obviously, suitable olefines from other sources may also be employed in the charging stock to the polymerizer.

In the catalytic polymerization of olefines, a mixture containing these reactive compounds is passed over a suitable catalyst at moderate to high superatmospheric pressure and at moderate temperatures. As catalysts, such materials as phosphoric acid on carbon, the solid obtained by calcining a mixture of phosphoric acid and kieselguhr (the so called solid phosphoric acid), copper pyrophosphate, copper orthophosphate plus cadmium orthophosphate plus phosphoric acid, sodium aluminum chloride, lithium aluminum chloride, antimonous aluminum bromide, mercuric aluminum bromide and similar contact agents have been suggested. Operating pressures of from 200 to 1500 pounds per square inch, more or less, have been suggested and temperatures of from 200° F. to 550° F., more or less. Specifically, excellent results have been obtained when operating at a temperature of 350° F. to 375° F. and a pressure of 1500 pounds per square inch, the olefine containing charge being passed over the catalyst at a rate of 20 cubic feet (measured at standard conditions) per hour per pound of catalyst.

Thus far in the discussion major emphasis has been placed on the polymerization of mixtures containing olefines having four carbon atoms to the molecule. Such olefines are most suitable

for polymerization. Ethylene polymerizes at a very slow rate and while in the presence of higher olefines the rate of ethylene polymerization is greatly accelerated, yet the use of this olefine is not recommended. Propene polymerizes at a satisfactory rate but tends to give considerable high boiling polymer. This can be prevented largely by conducting the polymerization in two or more steps with product separation between steps but obviously this greatly increases the cost of the apparatus. Isobutene is about ideal as a polymerization unit charge but perfectly satisfactory results may be obtained using an isobutene-normal butenes mixture and either limiting the amount of normal butenes polymerization or having an isobutene-normal butenes ratio of about one or more.

The polymer produced is separated from the gaseous components of the reaction mixture. These last are preferably recycled to the zone wherein paraffins are converted into olefines. The polymer is hydrogenated. This may be accomplished by subjecting a polymer-hydrogen mixture to a high superatmospheric pressure at moderately elevated temperatures in the presence of a relatively inactive but highly stable hydrogenation catalyst such as a sulfide or oxide of molybdenum or tungsten. Usually however the hydrogenation is accomplished under milder conditions, for example, 200 pounds per square inch pressure and a temperature of 400° F. to 600° F., more or less, in the presence of a more active catalyst, for example, nickel.

The blending of either the total hydrogenated polymer or any suitable fraction thereof with the higher boiling cut from the product of the destructive isomerization of a hydrocarbon fraction or any suitable fraction obtained from said higher boiling cut, to produce a motor fuel of high octane number; high lead response, high and controllable volatility and low unsaturate content is a procedure obvious to those skilled in the art.

For the better understanding of this invention reference may be had to the accompanying figure, forming a part of this specification, which is a diagrammatic representation of one form of apparatus suitable for use in accomplishing the objects of this invention.

Turning now to a more detailed consideration of the figure, suitable liquid charge of a nature previously described is moved by pump 1 through line 2 to the destructive isomerization reactor 3. A suitable catalyst, for example, aluminum chloride, is held in hopper 4 and is added to the liquid charge at a predetermined rate through valve 5, the addition being accomplished by means of an eductor or similar device. Reactor 3 is supplied with heating means, for example, coil 6 through which steam, hot oil, heated biphenyl, heated biphenyl-diphenyl oxide or the like may be circulated. An activator such as water, steam, hydrogen chloride, an alkyl chloride or the like may be supplied to reactor 3 at a predetermined rate through valved line 7. The reactor 3 may be provided with suitable agitation means (not shown) if desired.

Volatile reaction products leave reactor 3 through conduit 8 and pass to fractionator 9 which is conventional, being provided with means to promote liquid-vapor contact, for example, bubble trays 10, with bottom heating means, for example, heating coil 11 and upper disposed cooling means, for example, cooling coil 12. The volatile reaction products are fractionated in 9, isobutane being taken overhead through line 13, 75

partially condensed in exchanger 14 and sent to separator 15. Condensed isobutane is moved by pump 16. Part may be circulated through valved line 17 to tower 9 to provide open reflux therein. Net condensed isobutane passes through valved line 18 wherein it is mixed with uncondensed isobutane from valved line 19. The mixture passes to the catalytic dehydrogenation zone. Material boiling above isobutane but below liquid charge is removed from an intermediate point of tower 9 through line 20, to be utilized as will be explained. Bottoms falling within the boiling range of the liquid charge are removed from tower 9 through valved line 21 and are returned to reactor 3. Sludge and polymer are removed from reactor 3 at a predetermined rate through valved line 22.

Isobutane passes through valved lines 18 and 19 to line 23 and thence to coil 24 in furnace setting 25. If desired, natural gas butanes may be added to the isobutane stream via valved line 26. On passage through coil 24 the gas stream is heated to catalytic dehydrogenation temperature and is then passed to reactor 27 which, if desired, may take the form of an upper manifold 28, a lower manifold 29 and a plurality of connecting tubes 30. These tubes are filled with a suitable dehydrogenation catalyst, for example, chromium oxide on alumina and are preferably placed in a furnace setting to supply the endothermic reaction heat. Reaction products pass via line 31 to the bottom of absorber 32 wherein they are contacted with a descending stream of absorber oil introduced through 33. Absorber 32 is provided with means to promote liquid-vapor contact, for example, bubble trays 34. Gas, consisting essentially of hydrogen, is eliminated through valved line 35. Rich absorber oil is moved by pump 36 through exchanger 37 to stripper 38. Stripper 38 is provided with means to promote liquid-vapor contact, for example, bubble trays 39, and with bottom heating means, for example coil 40. Stripped absorber oil is moved by pump 41 through exchanger 37, cooler 42 and line 33 to absorber 32. Dehydrogenated products comprising isobutane and isobutene (plus normal butane and the normal butenes if natural gas was introduced through 26) are discharged from stripper 38 through line 43, are cooled and preferably liquefied in cooler 44 and are moved by pump 45 to coil 46 in furnace setting 47. If available, 64 hydrocarbons from cracking still gas may be introduced through valved line 48.

Catalytically dehydrogenated products are heated to catalytic polymerization temperature in coil 46 and are passed to reactor 49 wherein they are contacted with a polymerization catalyst, for example, copper pyrophosphate. Products pass via valve 50 (where some pressure reduction is accomplished) to fractionator 51 which is similar to tower 9. Olefine polymerate may be removed by line 52 and valved line 53 to line 54, or, if desired, an intermediate cut of olefine polymers may be removed via valved line 55 to line 54 while olefine polymer bottoms may be removed via line 52 and valved line 56, valve 53 being closed. Overhead from tower 51 is recycled via line 57 to the catalytic dehydrogenation zone. Conditions are regulated in the catalytic polymerization zone so as to achieve as nearly complete olefine conversion as is conveniently possible.

Polymer liquid in line 54 is brought to a catalytic hydrogenation pressure by pump 58 while hydrogen in line 35' is brought to a similar

pressure in compressor 59, the two streams being mixed in line 60 and sent through coil 61 in furnace setting 62. During passage through coil 61 the mixture is brought to catalytic hydrogenation temperature and is then sent to reactor 63 containing a suitable hydrogenation catalyst, for example, nickel on kieselguhr. Products leave reactor 63 by line 64, are cooled in 65 and pass to separator 66 from which hydrogen is removed via valved line 67 and is sent to compressor 59 for recycling. Hydrogenated liquids are removed from separator 66 via valved line 68, are heated in heater 69 and are sent to fractionator 70. If the polymer liquid was fractionated in tower 51, then tower 70 need do no more than stabilize the hydrogenated polymer fraction. However, if total polymer was hydrogenated, then the hydrogenated total polymer may be fractionated in 70. If desired, no fractionation need be done in either tower, but as a rule it is preferable to remove and discard heavy ends of the liquid, either before or after hydrogenation. Tower 70 is provided with means to promote liquid-vapor contact, for example, bubble trays 71, with bottom heating means, for example, heating coil 72 and with upper disposed cooling means, for example, cooling coil 73. Gas, consisting essentially of hydrogen, is taken overhead from tower 70 by line 74 and may be sent by valved line 75 to line 35' for recycling. If desired, prior to recycling, the gas may be purified, for example, by absorption, using if desired absorber 32. Any excess gas over requirements may be discharged through valved line 76. If desired, an intermediate cut of hydrogenated polymer may be removed through valved line 77, passed to line 78 and thence to line 20 to form the ultimate product by blending with the light isoparaffinic naphtha. In such a case tower bottoms may be discharged through valved line 79. Or, if desired, valves 77 and 79 may be closed and the total liquid charge to tower 70 may be removed by valved line 80, thence to line 78 and finally to line 20 wherein the material is blended with light isoparaffinic naphtha to form the ultimate product of the process.

For the better understanding of the instant invention the following examples illustrating the same are given. It is to be understood that these examples are illustrative only and in no way limit the scope of the instant invention.

#### Example 1

A heavy naphtha obtained from East Texas crude and having a boiling range of from 250° F. to 400° F. and a motor octane number of about 45 was mixed with about 1% aluminum bromide and the resulting material was passed continuously to a liquid phase reactor operating at about 210° F. Overhead from the reactor was partially condensed to produce a gaseous fraction comprising isobutane and a liquid fraction containing large amounts of isoparaffins and having a motor octane number of about 80. From time to time a very small amount of steam was added to the reactor to activate the catalyst. From time to time sludge was withdrawn from the reactor. The isobutane fraction from the destructively isomerized product was compressed to a pressure of about two atmospheres and was passed through a catalytic dehydrogenation zone containing a catalyst comprising chromium oxide mounted on alumina and heated to a temperature of somewhat above 1025° F. On charging the isobutane at a rate of about 250 cubic

feet (measured at standard conditions) per hour per cubic foot of reactor volume, a gaseous product containing 30% hydrogen, 40% unconverted isobutane, 25% isobutene and 5% of various minor components was obtained. This was subjected to absorption-fractionation to remove hydrogen and the resulting hydrocarbon mixture, having an olefine content of over 35% was compressed to 1500 pounds per square inch pressure and passed at 365° F. over a catalyst comprising solid phosphoric acid, the flow rate being 35 cubic feet of charge (measured at standard conditions) per pound of catalyst per hour. The product, after partial pressure release, was stabilized to eliminate hydrocarbons containing four carbon atoms to the molecule. These were mixed with isobutane from destructive isomerization and the mixture was passed to the above mentioned catalytic dehydrogenation zone. The polymer was mixed with the hydrogen eliminated from the previously mentioned absorption-fractionation zone, the mixture was compressed to a pressure of about 200 pounds per square inch and then hydrogenated at 600° F. in the presence of a nickel catalyst. The reaction mixture from the hydrogenation zone was separated, hydrogen being recycled and the hydrogenated polymer being blended with a sufficient amount of the light highly isoparaffinic naphtha produced in the destructive isomerization zone to give an aviation fuel of high octane number, high lead response, high and proper volatility and low unsaturate content. By adding tetraethyl lead to this blend it was easily possible to achieve 100 octane number with less than 3 cc. per gallon and well over 100 octane number with 6 cc. per gallon, this larger quantity of lead tetraethyl being permissible in some aviation fuels for military purposes.

#### Example 2

The procedure was similar to that described in Example 1 except that the isobutane, formed during the destructive isomerization of the East Texas heavy naphtha, was mixed with 1.5 times its volume of the butane cut from natural gas, containing 80% normal butane and 20% isobutane, prior to passage to the catalytic dehydrogenation zone.

#### Example 3

The procedure was similar to that described in Example 1 except that the isobutene-isobutane fraction, prior to passage to the catalytic polymerization zone was mixed with three volumes of a refinery gas fraction containing hydrocarbons of four carbon atoms and showing on analysis 15% isobutene and 30% normal butenes.

It is obvious that in all of the above examples operations are continuous, in other words, the appropriate materials are charged continuously and at suitable rates to the destructive isomerization zone, the catalytic dehydrogenation zone, the catalytic polymerization zone and the catalytic hydrogenation zone.

The foregoing description and examples serve to outline the scope and spirit of the present invention and manifest its advantages to those skilled in the art to which it pertains but it is not intended that these shall be regarded as limitations upon the scope of the invention except insofar as included in the accompanying claims.

I claim:

1. In the preparation of motor fuel, the steps comprising subjecting a heavy naphtha to de-

structive isomerization, separating the destructively isomerized product into a relatively low boiling fraction and a relatively high boiling fraction having a maximum boiling point lower than the initial boiling point of said heavy naphtha, dehydrogenating said relatively low boiling fraction with the production of olefines and hydrogen, polymerizing said olefines, hydrogenating the polymer produced and blending the resulting hydrogenated polymer with said relatively high boiling fraction.

2. In the preparation of motor fuel, the steps comprising subjecting a heavy naphtha to destructive isomerization, separating the destructively isomerized product into a relatively low boiling fraction and a relatively high boiling fraction having a maximum boiling point lower than the initial boiling point of said heavy naphtha, dehydrogenating said relatively low boiling fraction with the production of olefines and hydrogen, separating said olefines and said hydrogen, polymerizing said separated olefines, hydrogenating the polymer produced with said separated hydrogen and blending the resulting hydrogenated polymer with said relatively high boiling fraction.

3. In the preparation of motor fuel, the steps

comprising subjecting a heavy naphtha to destructive isomerization, separating the destructively isomerized product into a fraction comprising isobutane and a higher boiling fraction having a maximum boiling point lower than the initial boiling point of said heavy naphtha, dehydrogenating said fraction comprising isobutane with the production of isobutene and hydrogen, polymerizing said isobutene, hydrogenating the polymer produced and blending the resulting hydrogenated polymer with said higher boiling fraction.

4. In the preparation of motor fuel, the steps comprising subjecting a heavy naphtha to destructive isomerization, separating the destructively isomerized product into a fraction comprising isobutane and a higher boiling fraction having a maximum boiling point lower than the initial boiling point of said heavy naphtha, dehydrogenating said fraction comprising isobutane with the production of isobutene and hydrogen, separating said isobutene and said hydrogen, polymerizing said separated isobutene, hydrogenating the polymer produced with said separated hydrogen and blending the resulting hydrogenated polymer with said higher boiling fraction.

ROBERT F. RUTHRUFF.